

Aug. 31, 1937.

O. FRITZE ET AL

2,091,277

GASEOUS ELECTRIC DISCHARGE DEVICE

Filed Aug. 21, 1936



INVENTORS  
Otto Fritze  
Alfred Ruttenauer  
BY *Harry E. Dunham*  
ATTORNEY

## UNITED STATES PATENT OFFICE

2,091,277

## GASEOUS ELECTRIC DISCHARGE DEVICE

Otto Fritze, Berlin, and Alfred Ruttenauer, Berlin-Halensee, Germany, assignors to General Electric Company, a corporation of New York

Application August 21, 1936, Serial No. 97,294  
In Germany September 7, 1935

2 Claims. (Cl. 176—122)

The present invention relates to gaseous electric discharge devices generally and more particularly the invention relates to such devices having a luminescent material associated therewith which material emits light during the operation of the lamp to complement and supplement the visible light emitted by the luminescent gaseous electric discharge in the lamp.

Zinc silicate is a good luminescent material for use in connection with mercury vapor discharge lamps. Such material is usually manufactured for such use by first precipitating the material from a solution as a finely grained powder and then heating the material to a glowing temperature. It is usually necessary to heat such material to a glowing temperature several times before the material has the desired light output. During these heating periods the zinc silicate becomes coarse-grained and the grain size thereof ranges from about 1 to 300 mu and larger.

The object of the present invention is to provide a highly efficient gaseous electric discharge lamp having glowed zinc silicate associated therewith. Another object of the invention is to provide a lamp of this type which retains its high efficiency for a long useful operating life. A further object of the invention is to provide a gaseous electric discharge lamp having luminescent material associated therewith which may be transported in commerce with safety. Further objects and advantages attaching to the device and to its use and operation may be apparent to those skilled in the art from the following particular description.

We have discovered that the grain size of the zinc silicate has a great influence on the light output of a mercury vapor discharge lamp having a coating of zinc silicate on the container as well as on the loss of efficiency of the lamp during the operation thereof. We have discovered, further, that when the particles of zinc silicate have a grain size of between approximately 50 and 100 mu the light output of the lamp is about twice that of similar lamps in which the grain size of the zinc silicate ranges from 1 mu to 300 mu. The increased light output of the lamp of the present invention is due to the fact that the elimination of particles having a grain size less than 50 mu reduces the reflection of the light by the luminescent material. Further, when the coating is applied to the inner surface of the lamp container the elimination of the zinc silicate particles of less than 50 mu reduces the loss in light output of the lamp during the operation thereof since the larger particles of the zinc silicate have a

smaller surface as compared to their mass than the smaller particles and hence the light converting quality thereof is less impaired by the discharge during the operation of the lamp. We have demonstrated that the light output of a mercury vapor discharge lamp having a coating of zinc silicate on the inner surface of the container thereof in which the grain size of the zinc silicate particles is greater than 50 mu is three times that of a similar lamp in which an appreciable part of the zinc silicate coating consists of particles having a diameter smaller than 50 mu after both lamps have been operating for a period of approximately 100 hours.

The elimination of particles having a grain size greater than 100 mu is advantageous since particles of larger grain sizes are apt to drop off the container wall during transportation of the lamp. When desired, the particles of a grain size of about 50 to 100 mu are selected by sieving the glowed zinc silicate.

In the drawing accompanying and forming part of this specification an embodiment of the invention is shown in a side elevational, partly sectional view.

Referring to the drawing the lamp comprises an elongated tubular container 1 having an electrode 4 sealed therein at each end, which electrode 4 is connected to a current lead 3 sealed into the external pinch 2 of the container 1. Said container 1 has a gaseous atmosphere therein consisting of a starting gas, such as argon, at a pressure of approximately 1 to 10 mm. and a quantity 6 of vaporizable material therein, such as mercury, the vapor of which emits light during the operation of the device.

Said container 1 has a luminescent coating 5 of zinc silicate thereon the particles of which have a grain size of approximately 50 to 100 mu. The luminescent material is applied to the inner wall of said container by methods now known in the art, such as by first covering the inner surface of said container 1 with a volatile binder, such as a mixture of glycerin and alcohol, and then applying the zinc silicate particles, as by dusting, to the binding material. The binder is then volatilized and removed from the container 1, as by heating and exhausting said container 1. The electrodes 4 are electron emitting when heated and consist of a pulverized, sintered mixture of high melting point material, such as tungsten, and a material having high electron emissivity characteristics, such as an alkaline earth oxide.

A lamp having the structure described above

is a highly efficient light source, retains its efficiency for a long useful operating life and can be transported in commerce without particles of the luminescent material separating from the container wall.

While we have shown and described and have pointed out in the annexed claims certain novel features of the invention, it will be understood that various omissions, substitutions and changes 10 in the forms and details of the device illustrated and in its use and operation may be made by those skilled in the art without departing from the spirit and scope of the invention, for example, other types of thermionic electrodes, such 15 as the well known Hull type of hot, electron emitting electrode, or an electrode consisting of a bar or rod of electron emitting, oxide material having a filament of high melting point material, such as tungsten, wrapped around it, are used

in place of the electrodes 4, when desired, or cold electrodes are used, when desired.

What we claim as new and desire to secure by Letters Patent of the United States, is:—

1. A gaseous electric discharge lamp device 5 comprising a container, electrodes sealed therein, a gaseous atmosphere therein and a coating of zinc silicate associated with said lamp, said zinc silicate having a grain size from about 50 to 100 mu.

10 2. A gaseous electric discharge lamp device comprising a container, electrodes sealed therein, a gaseous atmosphere therein comprising mercury vapor and a coating of zinc silicate on the inner surface of said container, said zinc 15 silicate having a grain size from about 50 to 100 mu.

OTTO FRITZE.  
ALFRED RUTTENAUER.